

## UNITED STATES PATENT OFFICE

2,089,580

## CORROSION INHIBITOR

Walter A. Schulze, Bartlesville, Okla., assignor  
to Phillips Petroleum Company, Bartlesville,  
Okla., a corporation of Delaware

No Drawing. Application September 10, 1934,  
Serial No. 743,493

## 14 Claims. (CL 44—9)

This invention relates to the prevention of corrosion of metals, and refers more particularly to a new and improved treatment of hydrocarbon oils containing sulfur. It includes both the 5 method of treatment and the product obtained.

More specifically this invention relates to the treatment of hydrocarbon liquid fuels ranging from liquefied petroleum gases through kerosene to prevent or retard or inhibit the corrosive action 10 of elementary sulfur on such metals as copper, bronze, etc.

Gasolines as commercially produced always contain more or less elementary sulfur resulting from the oxidation or decomposition of hydrogen sulfide and/or organic sulfur compounds during fractionation or other heat treatment of these products. Furthermore, during the doctor sweetening operation wherein free sulfur is added to the oil for the purpose of converting the lead 15 mercaptides to lead sulfide and alkyl disulfides some excess of free sulfur must be used in order that the "breaking out" operation can be obtained in a reasonable amount of time. Therefore, regardless of how the oils are produced 20 some free sulfur is practically certain to be present and such sulfur reacts readily with copper and its alloys when the said oils are in contact with such metals.

Similar problems or disadvantages are met 25 with liquefied petroleum gases which is the name applied to a material similar to gasoline in physical properties but which consists largely of low boiling hydrocarbons such as propane and butane which are kept in the liquid state by the use of pressure. If such liquefied gases are drawn off in the vapor form then free sulfur will be concentrated in the containers and over a period of time the quantity may become quite large. It is common practice in dispensing liquefied petroleum 30 gases to use certain materials containing copper and its alloys, and such materials are particularly subject to corrosion by free sulfur. This corrosion and consequent weakening of the materials is especially dangerous where such elevated pressures are necessary.

At the present time it is necessary to treat the crude hydrocarbon products by very rigorous and expensive methods in order that the quantity of free sulfur present in the finished products is 35 sufficiently low that the rate of corrosion will not be exorbitant.

I have now discovered that by the addition of small amounts of certain compounds to the free sulfur containing hydrocarbon oils the corrosive 40 action of the sulfur on such metals as copper and

its alloys is prevented or retarded or inhibited. I have found that the organic compounds of the general formula  $\text{CH}_2\text{OH}-\text{CH}_2-\text{O}-\text{R}$  wherein R is either an alkyl, aryl, acyl or benzoyl radical, are particularly effective for this purpose. 5 Such compounds are generally referred to as the mono-alkyl or aryl ethers and esters of the glycols. I have discovered that ethylene glycol mono-ethyl ether is particularly outstanding in its effectiveness in preventing or retarding or inhibiting the action of free sulfur on copper.

Ethylene glycol is commonly thought to be insoluble in light hydrocarbon oils, nevertheless I have found that when a few drops of this compound is added to and/or left in contact with a 10 hydrocarbon oil containing free sulfur that such free sulfur does not corrode copper surfaces. I have found glycerin, also, to be effective for this purpose.

Other compounds such as propylene and butylene glycols and their mono-alkyl and aryl ethers and esters when added to hydrocarbon oils prevent or retard or inhibit the free sulfur in such oils from reacting with copper and its alloys. The derivatives of diethylene glycol and triethylene 20 glycol can likewise be used in this invention.

According to this invention a small amount of one of the compounds mentioned, e. g. ethylene glycol mono-ethyl ether, is added to a hydrocarbon oil containing elementary sulfur. In general the preferred actual concentration of the compound may vary between the limits of 0.001 25 percent to 0.1 percent. Such quantities give good results but larger or smaller amounts of the glycol compound may be used without departing 30 from the scope of this invention.

The amount of the glycol compound needed to prevent corrosion of the copper depends to some extent on the amount of free sulfur in the hydrocarbon solution. The percent of the compound to be used in the oil depends also on the ratio of the surface area of the copper to the 35 volume of the oil.

It is to be understood that the "corrosion-preventing" agent may be added either to a hydrocarbon oil already containing free sulfur or to an oil which may subsequently contain elementary sulfur as a result of the decomposition and/or the oxidation of unstable sulfur compounds 40 therein.

I have found that the various compounds are not equally effective and that much larger quantities of certain of the compounds must be used if equivalent effectiveness is to be obtained. The 45 results indicate (1) that in general the ethers 50

are more effective than the esters and (2) that the simple alkyl groups such as the methyl and ethyl are considerably better than the butyl or benzyl group.

- 5 One of the tests used for evaluating the effectiveness of these compounds is the corrosion test wherein a clean copper strip is immersed in the hydrocarbon oil and heated to 140° F. for several hours. The length of the heating period before 10 appearance of discoloration on the copper strip is the measure of the corrosiveness of the oil. Another test is merely that of noting the time during which no discoloration appears on the copper strip immersed in a naphtha solution at 15 room temperature.

The following examples will illustrate the practice of the invention:

- Example 1.—Fifty cc. of a naphtha containing 0.00086 percent elementary sulfur and 0.01 percent ethylene glycol mono-ethyl ether showed no discoloration on a copper strip even after heating for 3 hours at 140° F. An untreated sample was almost immediately corrosive to copper.

- Example 2.—0.00086 percent elementary sulfur was added to a freshly distilled light naphtha. A copper strip immersed in a 60 cc. portion of this naphtha was quite badly corroded after twenty minutes at room temperature whereas a copper strip immersed in a similar portion of the naphtha to which was added 0.002 percent ethylene glycol mono-ethyl ether showed no discoloration or corrosion at the end of 78 days.

- Example 3.—A 60 cc. portion of naphtha containing 0.00086 percent elementary sulfur gave a badly corroded copper strip at the end of fifteen minutes at room temperature whereas a similar portion of the naphtha to which was added approximately 0.014 percent of ethylene glycol mono-acetate had produced no discoloration on a copper strip when noted at the end of two days. After standing for 66 days the only corrosion evident constituted several tiny black spots about the size of pin points, really a negligible amount.

- Example 4.—A 60 cc. portion of naphtha containing 0.00086 percent elementary sulfur gave a badly corroded copper strip at the end of fifteen minutes at room temperature whereas a similar portion of the naphtha to which was added 0.024 percent of ethylene glycol mono-benzyl ether showed no discoloration on the copper at the end of 48 hours.

- Example 5.—A little ethylene glycol (0.014 percent by volume) was put into a bottle with a light naphtha containing 0.00086 percent elementary sulfur. No corrosion or discoloration could be detected on the copper strip after being immersed in the naphtha for ten days.

- Example 6.—A couple of drops of glycerin were placed in a bottle of naphtha containing 0.00086 percent elementary sulfur. A copper strip in this naphtha showed no discoloration at the end of 65 days.

- Example 7.—A drop of triethylene glycol was placed in a bottle of naphtha containing 0.00086 percent elementary sulfur. A copper strip in this naphtha showed no discoloration at the end of 17 hours. After 29 hours, however, several black spots had appeared.

- Example 8.—0.002 percent of ethylene glycol mono-butyl ether prevented corrosion of copper 70 in a naphtha solution containing 0.00086 percent

elementary sulfur indefinitely (more than 78 days) whereas 0.0018 percent of the butyl ether was hardly effective at all. However, a larger quantity of the butyl ether (0.024 percent) was sufficiently effective that only a little corrosion 5 was noted at the end of 48 hours.

In a similar test the benzyl ether was found to be several times as effective as the butyl ether.

It is not desired to limit the invention to the concentration of the treating agents given in 10 the above examples. Use may be made of higher or lower concentrations of any members of the classes of compounds mentioned herein and as a result thereof longer or shorter periods of preventing, retarding or inhibiting corrosion of copper and its alloys by elementary sulfur secured 15 depending upon the specific agent used, the concentration of the agent, the percentage of free sulfur in the material treated and the conditions under which the subsequent storage takes place. 20

Obviously these various glycol compounds differ greatly in their solubility in hydrocarbon oils. Some of them are practically insoluble while others are readily soluble. Inasmuch as the desired solubility can usually be obtained by the 25 introduction of "more oil soluble" or "less oil soluble" groups into such compounds, it is to be understood that such may be made without departing from the spirit and scope of this invention. Miscibility agents such as butyl alcohol 30 can likewise be added with the more insoluble compounds like ethylene glycol or glycerin to increase their solubility in the hydrocarbon oils.

I claim:

1. The method of inhibiting the corrosion of 35 copper and its alloys by hydrocarbon liquid fuels ranging from liquefied petroleum gases through kerosene, said liquid fuels containing sufficient elementary sulfur so that they tend normally to corrode copper and its alloys, which comprises 40 adding to the said liquid fuels a small amount of a compound of the structure

$$R-O-(CH_2)_m-(CH_2-O-CH_2)_x-(CHOH)_n-H$$
 45  
wherein R represents a member selected from the group consisting of the alkyl, aryl, acyl and benzoyl radicals and wherein x represents an integer from the group 0, 1 and 2 and m represents an integer from the group 1, 2 and 3 and n represents an integer from the group 1 and 2.

2. The method of inhibiting the corrosion of copper and its alloys by hydrocarbon liquid fuels ranging from liquefied petroleum gases through kerosene, said liquid fuels containing sufficient 55 elementary sulfur so that they tend normally to corrode copper and its alloys, which comprises adding to the said liquid fuels a small amount of a compound of the structure

$$R-O-(CH_2)_m-(CH_2-O-CH_2)_x-CH_2OH$$
 60  
wherein R represents a member selected from the group consisting of the alkyl, aryl, acyl and benzoyl radicals and wherein x represents an integer from the group 0, 1 and 2 and m represents an integer from the group 1, 2, and 3.

3. The method of inhibiting the corrosion of copper and its alloys by hydrocarbon liquid fuels ranging from liquefied petroleum gases through kerosene, said liquid fuels containing sufficient 70 elementary sulfur so that they tend normally to corrode copper and its alloys, which comprises adding to the said liquid fuels a small amount of a compound of the structure

$$R-O-(CH_2)_m-(CHOH)_n-H$$
 75

wherein R represents a member selected from the group consisting of the alkyl, aryl, acyl and benzoyl radicals and wherein m represents an integer from the group 1, 2, and 3 and n represents an integer from the group 1 and 2.

4. The method of inhibiting the corrosion of copper and its alloys by hydrocarbon liquid fuels ranging from liquefied petroleum gases through kerosene, said liquid fuels containing sufficient elementary sulfur so that they tend normally to corrode copper and its alloys, which comprises adding to the said liquid fuels a small amount of a compound selected from the group consisting of the mono-alkyl and mono-aryl ethers and esters of ethylene glycol.

5. The method of inhibiting the corrosion of copper and its alloys by hydrocarbon liquid fuels ranging from liquefied petroleum gases through kerosene, said liquid fuels containing sufficient elementary sulfur so that they tend normally to corrode copper and its alloys, which comprises adding to the said liquid fuels a small amount of ethylene glycol mono-ethyl ether.

6. The method of inhibiting the corrosion of copper and its alloys by hydrocarbon liquid fuels ranging from liquefied petroleum gases through kerosene, said liquid fuels containing sufficient elementary sulfur so that they tend normally to corrode copper and its alloys, which comprises adding to the said liquid fuels a small amount of ethylene glycol mono-acetate.

7. Predominantly hydrocarbon liquid fuels ranging from liquefied petroleum gases through kerosene containing sufficient elementary sulfur to tend normally to corrode copper and its alloys to which has been added as a corrosion inhibitor a small amount of a compound of the structure



wherein R represents a member selected from the group consisting of the alkyl, aryl, acyl and benzoyl radicals and wherein x represents an integer from the group 0, 1 and 2 and m represents an integer from the group 1, 2 and 3 and n represents an integer from the group 1 and 2.

8. Predominantly hydrocarbon liquid fuels ranging from liquefied petroleum gases through kerosene containing sufficient elementary sulfur to tend normally to corrode copper and its alloys to which has been added as a corrosion inhibitor a small amount of a compound of the structure



wherein R represents a member selected from the group consisting of the alkyl, aryl, acyl and benzoyl radicals and wherein x represents an integer from the group 0, 1 and 2 and m represents an integer from the group 1, 2 and 3.

9. Predominantly hydrocarbon liquid fuels ranging from liquefied petroleum gases through kerosene containing sufficient elementary sulfur to tend normally to corrode copper and its alloys to which has been added as a corrosion inhibitor a small amount of a compound of the structure



wherein R represents a member selected from the group consisting of the alkyl, aryl, acyl and benzoyl radicals and wherein m represents an integer from the group 1, 2, and 3 and n represents an integer from the group 1 and 2.

10. Predominantly hydrocarbon liquid fuels ranging from liquefied petroleum gases through kerosene containing sufficient elementary sulfur to tend normally to corrode copper and its alloys to which has been added as a corrosion inhibitor a small amount of a compound selected from the group consisting of the mono-alkyl and mono-aryl ethers and esters of ethylene glycol.

11. Predominantly hydrocarbon liquid fuels ranging from liquefied petroleum gases through kerosene containing sufficient elementary sulfur to tend normally to corrode copper and its alloys to which has been added as a corrosion inhibitor a small amount of ethylene glycol mono-ethyl ether.

12. Predominantly hydrocarbon liquid fuels ranging from liquefied petroleum gases through kerosene containing sufficient elementary sulfur to tend normally to corrode copper and its alloys to which has been added as a corrosion inhibitor a small amount of ethylene glycol mono-acetate.

13. Predominantly hydrocarbon liquid fuels ranging from liquefied petroleum gases through kerosene substantially free of unsaturated hydrocarbons containing sufficient elementary sulfur to tend normally to corrode copper and its alloys to which has been added as a corrosion inhibitor a small amount of a compound selected from the group consisting of the mono-alkyl and mono-aryl ethers and esters of ethylene glycol.

14. Liquefied petroleum gases containing sufficient elementary sulfur to tend normally to corrode copper and its alloys to which has been added as a corrosion inhibitor a small amount of a compound of the structure



wherein R represents a member selected from the group consisting of the alkyl, aryl, acyl and benzoyl radicals and wherein x represents an integer from the group 0, 1 and 2 and m represents an integer from the group 1, 2 and 3 and n represents an integer from the group 1 and 2.

WALTER A. SCHULZE. 60